

Patented Mar. 10, 1925.

1,529,299

# UNITED STATES PATENT OFFICE.

ALBERT L. CLAPP, OF DANVERS, MASSACHUSETTS

## FELT AND PROCESS OF MAKING THE SAME.

No Drawing.

Application filed May 10, 1922. Serial No. 559,960.

To all whom it may concern:

Be it known that I, ALBERT L. CLAPP, a citizen of the United States, residing at Danvers, in the county of Essex and State of Massachusetts, have invented new and useful Improvements in Felt and Processes of Making the Same, of which the following is a specification.

This invention has for its object to produce a compressible resilient felt, capable of use in the manufacture of gun wads, insulation for railway cars, ice houses, refrigerators and the like, and which is water-resistant and which moreover may be produced on a paper-making machine such as a "wet machine" so-called.

I first start with a cellulosic material,—preferably cotton linters so-called,—but in lieu of cotton linters I may use jute, rags or other suitable material. I load a beating engine with approximately 600 pounds of the cellulosic material, e. g., cotton linters; and, adjusting the roll to the bed plate, beat the raw material with sufficient water to ensure free circulation until the raw material is well beaten without material hydration. This takes ordinarily in the neighborhood of 4 hours more or less and effects a disintegration of the fibers. To the contents of the beater tub are added about 50 pounds of rosin size and the beating is continued until the rosin size is thoroughly incorporated in the mass, usually for about 1 hour. Then I add preferably aluminum sulphate in excess of that needed to precipitate the rosin size in the form of aluminum resinate. Ordinarily it would take about 25 pounds of alum to precipitate 50 pounds of rosin size, but preferably I add about 50 pounds of alum, thus providing an excess of 25 pounds. The beating is continued for about 1 hour until the aluminum resinate is precipitated on the fibers of the mass. The beater roll is then raised and about 600 pounds of cattle or goat hair (dry weight) derived from tanneries is added to the beater. The adjustment of the roll is such that, when the beater is again started in operation, the contents of the tub are thoroughly intermixed and the hair is brushed without cutting or hard beating. This may continue for about 1 hour. Wet hair from the tannery may be used or hair after it has been dried. In any event, such hair has usually mixed therewith more or less lime. (It is for this reason that I employ an excess of alum in the first sizing

of the mass, the excess alum serving to neutralize the lime and form soluble salts which wash out with the water.) The mass is then again sized by the addition of rosin size and sufficient alum to react therewith for the precipitation of aluminum resinate. For this purpose, I may add for example 20 pounds of rosin size and 10 pounds of alum, the latter of course being added after the rosin size has been thoroughly intermixed with the mass. The amounts of rosin size added at these different times to the mass of course may be varied. After the beating and brushing operations, the stock is then sheeted on a wet machine until the material on the make-up roll is of the desired thickness or caliper. The material is then stripped from the roll and is dried flat, after which it may be passed through calender rolls to compact the sheet slightly and to finish the surface of the sheet.

With not so good results, instead of a double sizing operation during the beating of the stock, the hair may be added to the beater after the cellulosic material has been properly beaten, and the rosin size added after the hair has been thoroughly intermixed with the cellulosic material during the brushing operation. Even in such case, because of the presence of lime in the cattle or goat hair, I use alum in excess of that necessary to react with the rosin size. In such case, after the cotton linters have been beaten for, say, 4 hours with hard beating, the rolls may be lifted and an equal amount of hair added. The beater is then set in operation and the mass is circulated and intermixed without cutting the hair for about 1 hour. I may then add 50 pounds of rosin size and continue the brushing operation for 1 hour, after which 75 pounds of alum may be added and the beater continued in operation for another hour. Preferably, when the alum is added, the roll is still further lifted to effect merely the circulation and intermixing of the components of the mass without an actual beating or brushing operation, since the final operation of the beater is merely to secure a thorough intermixing of all of the components of the stock. The pulp is then sheeted as previously described.

In some instances, instead of using cotton linters or jute or rags, I may substitute for all or a portion thereof such cellulosic material as chemical wood pulp,—or waste manila, rag or mixed papers,—or sulphite, sul-

phate or ground wood screenings,—this depending upon the particular use to which the felt is to be subjected.

The final product is water-resistant, 5 resilient and slow burning. When cut into blanks of the proper size, it may be used for the manufacture of dust guards, such as employed in railway car journals; or, as previously stated, it is excellent as a non-con- 10 ductor of heat and lends itself to use as an insulation for ice houses, railway cars, refrigerators, etc.

When cotton or other equivalent fiber is used as the initial or starting material, it 15 must be beaten to the required degree of fineness, as otherwise, on the addition of the hair which is only brushed, a stock would be produced which would be too free and more or less lumpy and would not properly form 20 or felt on the cylinder mold.

What I claim is:—

1. A soft compressible and resilient water-resistant felt comprising hair and cellulosic material in substantially equal parts in interfelting relation and containing a waterproofing precipitate, said material having the characteristics of one formed on a paper-making machine.

2. A method of producing a soft compressible water-resistant resilient felt which 30 comprises beating a cellulosic material, adding and intermixing therewith an approximately equal amount of tanners' hair with-

out materially cutting the hair, adding rosin size and sufficient alum to precipitate the 35 rosin size and to neutralize lime contained in the hair, and felting and sheeting the stock on a paper machine.

3. The herein described method of producing a water-resistant resilient compressible felt, which comprises beating cotton linters to disintegrate the fibers, then adding rosin size and alum in excess of that required to precipitate sodium resinate from the size, adding and intermixing waste tanners' hair with the stock without materially cutting the hair, the excess alum serving to neutralize the lime contained in the hair, then adding rosin size to the mass and precipitating aluminum resinate therefrom by 50 the addition of alum, and finally felting and sheeting the stock on a paper machine.

4. A method of producing a water-resistant fibrous material, which comprises beating a cellulosic material to effect a disintegration thereof, precipitating a size on the disintegrated fibers, adding and mixing waste tanners' hair with the mass to produce a substantially homogeneous mixture, precipitating a size throughout the mass, and 60 finally sheeting the mass on a paper machine.

In testimony whereof I have affixed my signature.

ALBERT L. CLAPP.